

## UNITED STATES PATENT OFFICE

WILLOUGHBY STATHAM SMITH, OF BENCHAMS, NEWTON POPPLEFORD, AND HENRY JOSEPH GARNETT, OF SEVENOAKS, ENGLAND

## MAGNETIC ALLOY

No Drawing. Application filed May 7, 1927, Serial No. 189,735, and in Great Britain July 27, 1926.

In the Patent No. 1,552,769 a number of alloys with high permeability with very weak magnetizing forces were described; amongst others, alloys composed as follows:

|           | No. 1 | No. 2 |
|-----------|-------|-------|
| Nickel    | 70.5% | 65%   |
| Iron      | 18.5% | 17%   |
| Copper    | 10.5% | 17%   |
| Manganese | 0.5%  | 0.5%  |

10 The first alloy had a magnetic permeability of 5300, and the second a magnetic permeability of 3200 in magnetic fields tending to zero.

15 According to this invention an alloy is composed of:

|        |        |
|--------|--------|
| Nickel | 69-71% |
| Iron   | 14-15% |
| Copper | 14-16% |

20 The magnetic permeability of such alloy, when suitably annealed (by heating to a temperature in excess of the magnetic change point and cooled so that its initial permeability is of the order of 6000) is almost independent of the strength of the field between  $H=.001$  and  $H=.1$  gauss. The alloy should be heated to a temperature of about  $880^{\circ}$  C. and air-cooled.

25 For example an alloy containing substantially:

|        |     |
|--------|-----|
| Nickel | 70% |
| Iron   | 15% |
| Copper | 15% |

30 with a trace of manganese, has given the following results when drawn to fine wire, annealed and tested:

$$\begin{aligned}
 H = .001 &= 6300 \\
 &= .01 = 6800 \\
 &= .05 = 7400
 \end{aligned}$$

35 The alloy has properties, therefore which make it, in a tape or wire form, very useful for the manufacture of loaded telegraphic and telephonic cables.

40 To the alloy may be added manganese in quantities of less than .5% as deoxidizer, but 45 should not contain any trace of carbon.

What we claim is:

1. A magnetic alloy comprising iron from 14 to 15%, copper from 14 to 16% and the remainder nickel, which has an initial magnetic permeability of the order of 6000 which permeability is substantially constant for various strengths of the magnetizing field. 55

2. A magnetic alloy comprising iron from 14 to 15%, copper from 14 to 16%, a de-oxidizing metal to an amount not greater than 0.5 and the remainder nickel, which has an initial magnetic permeability of the order of 6000 which permeability is substantially constant for various strengths of the magnetizing field. 60

3. A magnetic alloy comprising iron 15%, copper 15% and the remainder nickel, which has an initial magnetic permeability of the order of 6000 which permeability is substantially constant for various strengths of the magnetizing field. 65

4. A magnetic alloy comprising iron 15%, copper 15%, manganese to an amount not greater than 0.5% and the remainder nickel, which has an initial permeability of the order of 6000 which permeability is substantially constant for various strengths of the magnetizing field. 70

In testimony that we claim the foregoing as our invention we have signed our names to this twenty-fifth day of April, 1927.

WILLOUGHBY STATHAM SMITH.  
HENRY JOSEPH GARNETT.

85

90

95

100